

J. THOMSON.

METHOD FOR PREVENTING ELECTRIC CARBON RESISTERS FROM OXIDIZING.

APPLICATION FILED OCT. 7, 1918.

1,308,878.

Patented July 8, 1919.



INVENTOR

*John Thomson*  
BY  
*Kiddle Thomson*  
HIS ATTORNEYS.

# UNITED STATES PATENT OFFICE.

JOHN THOMSON, OF NEW YORK, N. Y.

## METHOD FOR PREVENTING ELECTRIC CARBON RESISTERS FROM OXIDIZING.

1,308,878.

Specification of Letters Patent.

Patented July 8, 1919.

Application filed October 7, 1918. Serial No. 257,213.

To all whom it may concern:

Be it known that I, JOHN THOMSON, a citizen of the United States, and a resident of the borough of Manhattan, city of New York, county and State of New York, have invented certain new and useful Improvements in Methods for Preventing Electric Carbon Resistors from Oxidizing, of which the following is a specification.

10 This invention relates to electric furnaces and consists in a method for preventing carbon resistors from oxidizing, or "air-burning".

15 The accompanying drawing is a diagrammatic sectional view of an electric furnace comprising the essential elements necessary to illustrate the present method. In said drawing a furnace construction is shown in which A is the base, B the side-walls, and 20 C the arched roof that together provide the furnace chamber D. Mounted in the side-walls, and passing through the chamber, is a carbon resistor E whose type is commonly designated as the "zig-zag", its terminals 25 being empirically shown in a power-circuit F.

Hitherto, the chief difficulty, and to a large extent the limiting factor, in the use of electric carbon resistors, irrespective of their 30 type or form, is their liability to attack and disintegration when air or other active gases are present in the resistor-chamber. A method has hitherto been employed to avoid the destruction of carbon resistors, as by the 35 introduction of an inert gas. For an example of such method see U. S. patent to F. A. J. Fitzgerald, No. 950,905, dated March 1, 1910. Said method has proven fairly successful; but the method now to be 40 described is more generally applicable in present practice and possesses certain important advantages.

Thus, the method now to be described consists of locating within a resistor-chamber 45 a charge composed of a mixture of oxid of zinc ( $ZnO$ ) and carbon (C), which, when sufficiently heated, reacts according to the classical formula,



50 If or when any oxygen is present in the resistor-chamber, it combines with the zinc-fume and produces  $ZnO$ , whereby the resistor itself is made wholly immune to pernicious attack; or, as expressed in common parlance, is immune to "air-burning".

The mixed charge, as *h*, may be conveniently introduced to the resistor-chamber, from time-to-time, through an opening or tube, as *m*, to be received by a pan, as *n* resting upon the resistor, or it may be dropped upon the bottom of the chamber, as at *r*. The tube may also be utilized as a vent, as at *s*, whereat to burn a flame of mixed or intermingled Zn-fume and CO, thereby indicating to an operator that the chamber contains an adequate supply of the benign vapor and gas.

It is preferable, for the present purpose, that both the zinc oxid  $ZnO$  and the carbon 70 C which compose the charge shall be of a high degree of purity, whereby the residuum of the reaction shall be a merely nominal amount; and also in that there shall be practically no other development of vapor and 75 gas than pure zinc-fume and monoxid of carbon.

Obviously, the charge needs not be located precisely within the confines of the resistor-chamber; for, if desirable, it might be placed 80 in a communicating side-chamber, or niche, or wherever sufficient heat could be directed thereon to produce the reaction; which becomes active at or about 1,000° C.

The following controlling advantages reside in the production of zinc-fume by means of the aforesaid reaction rather than by merely vaporizing metallic zinc: Firstly, the CO performs the function of an active carrier for the denser  $Zn$  vapor or fume and 90 serves to convey the latter into any crevices in the furnace-walls whereat, if air is present, it will burn to  $ZnO$ , thus automatically closing the vents and excluding a further entrance of oxygen. Secondly, the expansion 95 of the fume and gas, particularly when the resistor chamber is wholly inclosed, produces pressure, of which but a nominal amount is necessary to cause the reaction to cease. Consequently, when there are no vents to 100 permit escape of the fume and gas, or when no oxygen is present to consume the fume, the reduction of the charge is automatically suspended; and, *per contra*, if vents develop, and if air again enters, the benign reaction 105 is automatically resumed. In these circumstances, a merely nominal quantity of reacting charge serves to protect the resistor for a relatively long period of time. In fact, carbon resistors have been thus continuously 110 operated, at high temperatures, for periods of months, without the slightest deteriora-

tion; the conditions of service being such that, without the utilization of this method, they would not have endured but a few hours.

5 While the foregoing matter has preferably dealt specifically with the metallic vapor produced from oxid of zinc and the gas resulting from its reagent, monoxid of carbon, the method, broadly, is not necessarily confined 10 to these specific substances, in that the oxid of any metal, when combined with any suitable reagent whose reaction will produce a metallic vapor which combines with oxygen, and a gas which will not attack carbon, 15 may be utilized.

What I claim is:

1. In electric furnaces, the method of preventing a carbon resister from oxidizing which consists in locating a charge of oxid 20 of zinc and carbon (ZnO and C) within the resister-chamber and heating the said charge until it reacts and produces zinc fumes and carbon monoxid (Zn and CO.)

2. In electric furnaces, the method of preventing a carbon resister from destructive 25

attack, as from oxygen, which consists in filling the resister-chamber with vaporized zinc and monoxid of carbon.

3. In electric furnaces, the method of maintaining a gaseous mixture, composed of 30 zinc fumes and carbon monoxid (Zn and CO), which method consists in so situating a charge of oxid of zinc and carbon (ZnO and C) within a resister-chamber, that the ingredients of the charge will be caused to 35 react until the developed pressure is sufficient to automatically suspend the reaction.

4. In electric furnaces, the method of preventing a carbon resister from oxidizing which method consists of enveloping the resister in an atmosphere composed of the fumes or vapors from a vaporized metallic oxid and its gaseous reducing reagent.

This specification signed and witnessed this 13th day of September, A. D. 1918.

JOHN THOMSON.

Signed in the presence of—

RALPH M. THOMSON,  
H. O. WEED.